

April 29, 1947.

A. F. MITTERMAIER

2,419,847

POWDERED IRON MAGNETIC CORE

Filed June 2, 1944



Inventor:  
Armin F. Mittermaier,  
by Harry E. Dunham  
His Attorney.

## UNITED STATES PATENT OFFICE

2,419,847

## POWDERED IRON MAGNETIC CORE

Armin F. Mittermaier, Fort Wayne, Ind., assignor to General Electric Company, a corporation of New York

Application June 2, 1944, Serial No. 538,482

6 Claims. (CL. 175—21)

1

My invention relates to powdered iron bonded magnetic cores, and to an improved method of making such a core.

It has been customary to form electromagnetic cores particularly for high frequency application of powdered iron which is bonded together with suitable material, such as a phenolic condensation product, varnishes, chrome silicate, and waxes. The iron particles have also been insulated from each other by mixing the powdered iron with an insulating material such as clay before the powder is bonded together with a binder. Cores which I formed according to past practice, however, by the use of high pressure had relatively high core losses and were not consistent in electrical characteristics.

It is therefore an object of my invention to provide an improved powdered iron bonded core.

Another object of my invention is to provide an improved method of forming a powdered iron bonded core.

Further objects and advantages of my invention will become apparent from the following description referring to the accompanying drawing, and the features of novelty which characterize my invention will be pointed out with particularity in the claims annexed to and forming a part of this specification.

In the drawing, Fig. 1 illustrates a mold apparatus in which my improved core is formed; Fig. 2 illustrates a core produced in the mold of Fig. 1; Fig. 3 illustrates a modified mold construction for producing a modification of the core illustrated in Fig. 2, and Fig. 4 illustrates the core produced in the mold of Fig. 3.

My improved core is formed by mixing powdered iron of suitable fineness with a suitable insulating material such as clay. The clay is employed so as to prevent relative high eddy currents, but if the eddy currents are not material the clay or similar insulating material may be omitted. The mixture of powdered iron and clay is then mixed with any suitable heat hardenable substantially solventless liquid binding material such as esters of saturated monohydric alcohols and unsaturated monobasic carboxylic acid. Further examples of such materials are given in applications for Nordlander and Hargraves, S. N. 302,164, and Nordlander, S. N. 302,165 and S. N. 302,166. These further examples are listed below as follows:

S. N. 302,164

Polymerizable compositions comprising (1) a polymerizable polyhydric alcohol ester of an

alpha-unsaturated alpha, beta-polycarboxylic acid, e. g., diethylene glycol maleate, diethylene glycol fumarate, etc., and (2) a polymerizable monohydric alcohol ester of an alpha-unsaturated alpha,beta-polycarboxylic acid, e. g., diethyl fumarate, dipropyl itaconate, diallyl maleate, diallyl itaconate, etc.

S. N. 302,165

10 Polymerizable compositions comprising (1) a polymerizable polyhydric alcohol ester of an alpha-unsaturated alpha,beta-polycarboxylic acid and (2) a polymerizable polyester obtained by esterifying an aromatic polycarboxylic acid or anhydride with an unsaturated monohydric alcohol, e. g., diallyl phthalate.

S. N. 302,166

20 Polymerizable compositions comprising (1) a polymerizable polyhydric alcohol ester of an alpha-unsaturated alpha,beta-polycarboxylic acid and (2) an unsaturated monohydric alcohol triester of a tribasic acid, specifically triallyl phosphate, triallyl citrate, triallyl tricarballylate or triallyl aconitate.

25 In order to produce a finished core which will not be rubbery, I have found that it is desirable to use a suitable amount of catalyst with the solventless bonding material, that is, about 3 per cent by weight of the total amount of bonding material employed. Any suitable catalyst may be employed such as a peroxide such as benzoyl peroxide. Any suitable proportions of powdered iron insulating material and solventless binder may be employed and I have found that a mixture including about 8 parts of clay, 66 parts iron, and 26 parts binder produces a very desirable core.

30 In Fig. 1 I have illustrated somewhat diagrammatically a mold having similar portions 10 and 11 which fit into a base 12, in which mold the materials described above may be poured from a vessel 13 to produce a core. In order to insure that the mixture will fill all parts of the mold, 35 the mixture is preheated before introducing into the mold to a temperature just below the polymerization temperature of the resin binder, and for the materials mentioned above the mixture is heated to about 80 degrees C. for about 5 minutes while it is being agitated. The mixture is then poured into the mold to produce the core. In order to prevent the mixture from chilling when it is poured into the mold, the mold is preheated to at least the temperature that the mixture has, such as around 90 to 100 degrees by the

use of heating coils 14 and 15. The mold is maintained at the temperature of about 100 degrees for a few minutes and then raised to above the polymerization temperature of the binder, such as being raised to about 130 degrees for a suitable time such as 1 hour. After the mold has cooled the two halves 10 and 11 may be disassembled leaving a core 16 as is illustrated in Fig. 2.

I have found that the resulting core formed in the manner described above has better electrical characteristics than a similar core formed of powdered iron bonded together with chrome silicate. Tests of such cores were made by connecting the primary of a transformer having the powdered iron core in series with a capacitance to form a series resonant circuit and the highest voltage induced in the secondary winding of the transformer which also surrounded the core was measured. The transformer core having the powdered iron bonded together with chrome silicate was formed by mixing 300 mesh powdered iron with sufficient chrome silicate, the core being hardened under heat and pressure. A transformer having such a core when tested in the resonant circuit described above had a maximum induced voltage in the secondary of about 10,000 volts, while a transformer having a core formed according to my invention with a similar amount of powdered iron had a maximum induced voltage in the secondary of about 18,000 volts. It will be appreciated that the difference in voltages is a measure of the relative efficiencies of the two types of cores, and my improved core was therefore considerably more efficient.

Not only will my improved core have efficient electrical characteristics, but by casting the ingredients in the manner described above, suitable slots 17 may be placed in the outer surface of the core for the reception of a winding such as the low voltage primary winding turns. It will be seen that the mold sections 10 and 11 have their inner surfaces suitably slotted so as to produce the winding slots in the outer surface of the core, as is illustrated in Fig. 2. If winding slots are desired in a powdered iron core formed according to past practice by the application of pressure, not only is a much more electrically inefficient core produced but the core will be formed first with a cylindrical surface, after which the core is machined to produce the slots, and unless the powdered iron is bonded very solidly together the ridges between the slots may crumble.

A winding if desired may be cast into the core formed according to my invention, and in Fig. 3 I have illustrated a mold having portions 18 and 19 filled with a mixture of iron, clay and solventless binder, as is described above. The mixture is, of course, heated and before it hardens a winding 20 is inserted so as to be cast into the core. Instead of introducing the winding 20 into a heated mixture in the mold, the winding may be previously inserted in the mold and then the mixture poured in and then polymerized around the winding. Fig. 4 illustrates a core 21 formed with the winding 20 cast therein.

Although I have shown and described particular embodiments of my invention, I do not desire to be limited to the particular embodiments described, and I intend in the appended claims to cover all modifications which do not depart from the spirit and scope of my invention.

What I claim as new and desire to secure by Letters Patent of the United States is:

1. A mechanically strong uncompressed magnetic core material comprising particles of powdered magnetic material bonded together by a polymerized alcohol ester of carboxylic acid.

5 2. A hard mechanically strong pressure free low loss magnetic core casting comprising a mixture of powdered magnetic material and powdered insulating material bonded together by a polymerized polyhydric alcohol ester of an alpha-unsaturated alpha,beta-polycarboxylic acid and a catalyst.

10 3. A hard mechanically strong gravity compacted low loss magnetic core casting comprising, by weight, substantially 66 parts powdered iron, 26 parts binder and 8 parts clay, said binder comprising, by weight, substantially 97 parts polymerized polyhydric alcohol ester of alpha-unsaturated alpha,beta-polycarboxylic acid and 3 parts catalytic peroxide.

15 20 4. A hard mechanically strong gravity compacted low loss magnetic core casting comprising, by weight, substantially 66 parts powdered iron, 26 parts binder and 8 parts clay, said binder comprising, by weight, substantially 97 parts polymerized polyhydric alcohol ester of an alpha-unsaturated alpha,beta-polycarboxylic acid and a polymerizable monohydric alcohol ester of an alpha-unsaturated alpha,beta-polycarboxylic acid and 3 parts benzoyl peroxide as a catalyst.

25 30 5. A hard mechanically strong gravity compacted low loss magnetic core casting comprising, by weight, substantially 66 parts powdered iron, 26 parts binder and 8 parts clay, said binder comprising, by weight, substantially 97 parts polymerized polyhydric alcohol ester of an alpha-unsaturated alpha,beta-polycarboxylic acid and a polyester obtained by esterifying an aromatic polycarboxylic acid or anhydride with an unsaturated monohydric alcohol and 3 parts benzoyl

35 40 45 peroxide as a catalyst.

6. A hard mechanically strong gravity compacted low loss magnetic core casting comprising, by weight, substantially 66 parts powdered iron, 26 parts binder and 8 parts clay, said binder comprising, by weight, substantially 97 parts polymerized polyhydric alcohol ester of an alpha-unsaturated alpha,beta-polycarboxylic acid and an unsaturated monohydric alcohol triester of a tribasic acid and 3 parts benzoyl peroxide as a catalyst.

ARMIN F. MITTERMAIER.

#### REFERENCES CITED

The following references are of record in the 55 file of this patent:

#### UNITED STATES PATENTS

| Number       | Name           | Date           |
|--------------|----------------|----------------|
| 2,230,228    | Bandur         | Feb. 4, 1941   |
| 60 1,982,689 | Polydoroff     | Dec. 4, 1934   |
| 2,273,891    | Pollack et al. | Feb. 24, 1942  |
| 2,195,362    | Ellis          | Mar. 26, 1940  |
| 1,867,362    | Lathrop        | July 12, 1932  |
| 1,881,711    | Lathrop        | Oct. 11, 1932  |
| 65 2,043,346 | Buckley        | June 8, 1936   |
| 2,330,590    | Kaschke        | Sept. 28, 1943 |
| 1,948,308    | Neighbors      | Feb. 20, 1934  |
| 1,994,534    | Robinson       | Mar. 19, 1935  |

#### FOREIGN PATENTS

| Number  | Country | Date          |
|---------|---------|---------------|
| 647,072 | French  | July 24, 1928 |